

1

2,938,778

## AMMONIUM NITRATE GAS-GENERATING COMPOSITION

Jack Linsk, Highland, Ind., assignor to Standard Oil Company, Chicago, Ill., a corporation of Indiana

No Drawing. Filed June 21, 1955, Ser. No. 517,077

6 Claims. (Cl. 52—5)

This invention relates to a composition for the generation of a gas; and pertains, more particularly, to an improved gas-generating composition comprising ammonium nitrate as the primary gas-producing component of the composition, intimately mixed with a combustible binder material consisting essentially of plasticized polyvinyl acetate. Such composition is useful for the propulsion of rockets for ground-to-ground missiles, ship-to-shore missiles, air-to-ground missiles and air-to-air missiles and the compositions may also be used as propulsion means in "assist take-off" of military and commercial aircraft.

Ammonium nitrate is widely used as a component of high explosives, particularly the so-called safe explosives. Even though ammonium nitrate is classified as a high explosive, it is extremely insensitive to ordinary heating and to shock and cannot readily be detonated by the local application of heat or by a blasting cap. Further, when ignited, ammonium nitrate alone does not burn uniformly and has a tendency to go out. In order to improve the burning quality, to utilize the excess free oxygen available from the decomposition of the ammonium nitrate, and to provide shaped grains suitable for use in rocket motors and assist take-off motors, combustible binder material is used in the ammonium nitrate composition.

The use of ammonium nitrate base compositions as solid propellants for rockets and assist take-off units is attractive because of the cheapness and availability of ammonium nitrate, because of the relatively low flame temperature of decomposition of ammonium nitrate, that is, between about 3150° and 2900° F. and because of the availability of the excess free oxygen. The physical characteristics of ammonium nitrate and grain material produced therefrom introduce problems with respect to choice of binder components. Thus solid ammonium nitrate exists in different crystalline forms at different temperatures, the transition from one form to a different form involving a volume change of the ammonium nitrate. Volume changes which occur at about 90° F. and also at about 0° F. involve 3.5% and about 3% increase, respectively. It would therefore appear that an ammonium nitrate-base composition could be seriously affected by storage under the variable temperatures encountered in many parts of the world.

One requirement for a solid propellant grain suitable for military use is that it be ballistically stable after prolonged storage at temperatures as high as 170° F. or as low as —75° F. Another requirement is that the grain not shatter, crack or malperform ballistically after being subjected to temperature extremes; that is, 175° F. followed immediately by transfer to a cold box held at —75° F. in a series of at least two repeated cycles. Another severe requirement imposed on solid propellant grains is ignition at temperatures down to —75° F. with the same igniter charge which is suitable at ambient temperatures. Grains must also be able to withstand shattering at low temperatures and distortion at high temperatures when subjected to shock.

An object of this invention is the preparation of a gas-

2

generating composition using ammonium nitrate as the principal gas-generating material. Another object of the invention is the preparation of a shaped propellant composition (grain), consisting essentially of ammonium nitrate, a binder material consisting essentially of polyvinyl acetate plasticized with a plasticizer comprising at least one nitro aromatic compound, and a combustion catalyst, which grain is dimensionally stable and non-fissuring in the temperature range between about 175° F. and —75° F. Still another object is to produce a gas-generating composition comprising ammonium nitrate, a binder material consisting essentially of plasticized polyvinyl acetate, and an inorganic combustion catalyst, which gas-generating composition is suitable for use in rockets and assist take-off units. Yet another object is the preparation of a composition which is suitable for use as a binder for a mixture of ammonium nitrate and a combustion catalyst. A further object is to provide an improved grain which is useful as a rocket fuel and as fuel for a jet assisted take-off unit. This grain is characterized by having a burning rate at 1000 p.s.i., of at least 0.10 inch per second and which is preferably of the order of 0.10 to 0.20 inch per second or more, and a pressure exponent preferably below about 0.7. Other objects will be apparent as the detailed description of the invention proceeds.

The composition of the invention comprises ammonium nitrate, a combustion catalyst, and the binder material. The composition contains on a weight basis from about 70% to about 90% of finely ground ammonium nitrate, from about 1% to about 5% of a combustion catalyst, from about 0.2 to about 3% of an alkaline-reacting gassing inhibitor as described hereinbelow, and from about 5% to about 25% of combustible binder material. The binder contains at least about 20% of a solid polyvinyl acetate resin, usually from about 20% to about 60% by weight, the remaining components comprising at least one plasticizer material for the polyvinyl acetate, said plasticizer material containing at least one nitro aromatic compound as defined hereinbelow. Other components such as finely divided carbon may be added to the grain composition to improve the burning rate, reduce the pressure exponent, or improve low temperature ignitability.

The polyvinyl acetate resins employed in the binder material of this invention are transparent solid vinyl acetate homopolymers of relatively high molecular weight, preferably pulverized to pass through a #16 U.S. Standard mesh screen. The resins do not have sharp melting points. The lowest molecular weight polyvinyl acetate resins suitable for use as base material for the binders of this invention show softening points above about 190° C. Decomposition begins at temperatures of 200° C. to 250° C. These polymers have a specific gravity of about 1.20 at 20° C.

The viscosity of the homopolymers in general lies within the range of from about 50 to about 900 centipoises. For purpose of this specification and the claims based thereon, the term "viscosity" is defined as viscosity in centipoises of a benzene solution containing 86 grams of the resin per 1000 cc. of solution determined at 20° C. with an Ostwald viscosimeter.

The composition of the gas-producing propellant grain of this invention is substantially as follows:

|                                     | Percent    |
|-------------------------------------|------------|
| Ammonium nitrate                    | 70 to 90   |
| Plastic binder                      | 5 to 25    |
| Inorganic combustion catalyst       | 1 to 5     |
| Alkaline-reacting gassing inhibitor | 0.2 to 3.0 |
| Carbon                              | 0 to 5     |

To the composition may also be added a surfactant in an amount of 0.05% to 2.0% by weight to improve wet-

ting of the nitrate by the components and to improve the extrudability of the composition. The sorbitan oleates have been found to be effective for this purpose.

The plastic binder of this invention consists essentially of 20% to about 60% by weight of polyvinyl acetate, defined hereinabove, plasticized with 80% to 40% by weight of a plasticizer of which plasticizer at least 30% by weight and preferably at least 50% consists of nitro-substituted aromatic compounds, the remainder consisting of non-nitro containing material of variable oxygen content.

The term "ammonium nitrate" as used in this specification and in the claims is intended to mean either ordinary commercial grade ammonium nitrate such as conventionally grained ammonium nitrate containing a small amount of impurities which may be coated with a small amount of moisture-resisting material such as petroleum or paraffin; or to mean military grade ammonium nitrate or mixtures of minor amounts (usually less than 10%) of other inorganic nitrates such as sodium nitrate or potassium nitrate with the ammonium nitrate. A mixture of finely ground and coarsely ground ammonium nitrate is preferred, and the major proportion of the ammonium nitrate is finely ground. I prefer to grind the ammonium nitrate with a part or all of the catalyst component of the composition.

The binder of the gas-producing propellant composition is a thermoplastic material consisting of polyvinyl acetate blended with a plasticizer consisting of about 30% by weight (based on the binder) of one or more of a group of nitro-substituted aromatic compounds. This group includes dinitrobenzene, dinitrotoluene, and certain nitro-substituted aromatic ethers. Examples of these ethers are 2,4-dinitrophenyl ether and the di(dinitrophenyl)-polyglycol ethers. These are made via the Williamson reaction by reacting 2,4-dinitrochlorobenzene with phenol or glycols as taught in the copending application of Wayne A. Proell and Norman J. Bowman entitled "Thermoplastic Compositions" filed October 27, 1954, Serial No. 465,132. Other nitro ethers which may be used are dinitrophenyl propyl ether and dinitroanisole. The preferred class of nitro-substituted aromatic compounds corresponds to the general formula



where R is selected from the class consisting of hydrogen, methyl, nitrophenyl, phenoxy, mononitrophenoxy and alkoxy containing 1 to 4 carbon atoms.

In the choice of plasticizer components for the ammonium nitrate preference is reserved for highly oxygenated materials, other factors being equal. It is desirable to use at least one non-nitro containing plasticizer material. This can be an ester of a polyhydric alcohol or polycarboxylic acid. Examples are dialkyl phthalates, triethyl citrate, tributyl citrate, dialkyl diglycolates, diethyl and dibutyl tartrate, the Flexols, e.g., triethylene glycol di-2-ethylbutyrate, also known as triglycol dihexoate (Flexol 3GH), triglycol dioctanoate, (Flexol 3GO) and polyglycol dioctanoate (Flexol 4GO). These commercial "Flexol" products are fully described by Buttry in "Plasticizers" (1950) pages 49 and 50. The liquid plasticizer must be compatible with the polyvinyl acetate and the nitroaromatic components in the ratio used. Oxygen balance is important and esters of higher oxygen content are preferred when they have no undesirable effects. Some plasticizers impart good properties with regard to cycling, impact resistance, and hot aging, and these will be preferred regardless of oxygen balance.

Combinations of the above nitro compounds either alone or with the addition of other plasticizers produce

satisfactory polyvinyl acetate binders which are thermoplastic. When such binders are mixed with ammonium nitrate, grains may be fabricated which exhibit good resistance to shock and deformation at low or high temperatures. In general, liquid plasticizers for polyvinyl acetate are used only in conjunction with one or more nitro compounds in making binders suitable for use in solid propellant grains.

Cognizance of the stoichiometric oxygen balance is of importance in the choice of plasticizer material. Plasticizers which provide a substantial part of the oxygen requirement are preferred, since substantially smokeless combustion of the explosive grain composition is highly desirable. Coplasticizers with the nitroaromatic plasticizers preferably contain high oxygen balance. I prefer to use at least one plasticizer material not containing aromatic nitro groups. The non-nitro group containing plasticizers are preferably selected from the class consisting of esters of polyhydric alcohols and esters of polycarboxylic acids. Combinations of plasticizers such as dinitrotoluene with 2,4-dinitrophenyl ether and combinations of these with dinitrophenyl propyl ether with or without the addition of the non-nitro group-containing plasticizer components produce with the solid polyvinyl acetate very satisfactory thermoplastic binder material, which when used in the formulation of solid propellants containing ammonium nitrate, results in the production of grains which exhibit excellent resistance to shattering and deformation when subjected to shock at low or high temperatures. Such grains are found not to be altered with respect to burning properties after being subjected to such shock.

The relative amounts of the different plasticizers in the binder material may be varied over a wide range. Thus the plasticizer may consist entirely of 2,4-dinitrophenyl ether or may consist entirely of di(dinitrophenyl)-polyglycol ether, or other nitro compounds such as 2,4-dinitrotoluene may be used with the dinitrophenyl ethers. Likewise, variable amounts of dinitrophenyl propyl ether may be used along with these other nitro compounds. In general, other known plasticizers for polyvinyl acetate containing no nitro groups, such as the dialkyl phthalates and the Flexols, should be used only in conjunction with the nitro compounds as plasticizers for the polyvinyl acetate in the binder material.

The inorganic combustion catalyst of this invention is selected from the class consisting of ammonium dichromate and Prussian blue. Certain iron compounds broadly designated as Prussian blue are effective for the combustion of ammonium nitrate grains containing oxidizable binder materials. These catalysts are the subject matter of U.S. patent application filed by Wayne A. Proell and William G. Stanley, S.N. 273,564 and S.N. 288,065, filed May 15, 1952, now abandoned. Mixtures of ammonium dichromate with insoluble Prussian blue may be used. In general, ammonium dichromate tends to give lower pressure exponents and hence the inorganic catalyst should consist at least partially of ammonium dichromate. However, an inorganic catalyst consisting essentially of insoluble Prussian blue may be used.

One of the requirements of the solid propellant composition is chemical stability at relatively high temperatures. This is related to the gassing tendency as measured by the "135° C. gas stability test," which test is described hereinbelow. The ammonium nitrate solid propellants based on polyvinyl acetate binders require an inhibitor component in order to reduce gassing of the compositions under relatively high temperature storage conditions. The inhibitors which give satisfactory results are in general alkaline reacting. It has been found that certain amines are particularly effective, for example, 1,3-diaminobenzene, diphenylamine and urea. However, I prefer magnesium oxide as the gassing inhibitor for these compositions. As indicated hereinabove, these gassing inhibitors are utilized in amounts within the range of from

about 0.2% to about 3% by weight of the gas-producing composition.

Finely divided carbon may be added to the gas-producing composition in amounts up to about 5% by weight, preferably in amounts of 0.5 to 2.0% by weight of the finished grain for the purpose of improving burning rate. Highly adsorptive activated carbons such as "Norit" and "Nuchar" make up one class of effective burning rate additives. A second general type of carbon useful for increasing the burning rate of compositions are the carbon blacks, roughly classified as the channel blacks and the furnace combustion blacks. The carbon blacks are characterized by low ash content, and by having extremely small particle size, that is, 50 to 5000 Å. In order to avoid dusting and afford convenience in handling, some carbon blacks are available in "bead" form. The "beads" are extremely soft and disintegrate during the mixing of the composition. Examples of "bead" type carbon blacks are Micronex beads (channel blacks) and Statex beads (furnace blacks).

A third type of carbon which may be used in the composition is finely ground petroleum coke, particularly petroleum coke obtained as residue in the pipe-stilling of mid-continent heavy residuums. Such coke usually contains less than about 1% ash and hence, like the carbon blacks, is particularly suitable in gas-producing grains where it is desirable to keep to a minimum solid inorganic particles in the combustion gas. The coke may be activated by methods well known in the art to improve the efficiency thereof as a burning rate promoter and it is preferably ground to pass through a #325 U.S. Standard sieve.

Preparation of the compositions of this invention consist of these three steps: making the binder, mixing binder with ammonium nitrate and other ingredients to form a homogeneous solid composition, and molding the finished solid propellant grain. The binder is prepared by adding polyvinyl acetate to a mixture of nitro compounds and plasticizer at 120-150° C. in a suitable mixer. Mixing is continued until the polyvinyl acetate is completely plasticized. This occurs readily. Blending of the binder with ammonium nitrate and the other components of the formulation may be carried out in the same mixer if desired. A mixing temperature of 90-105° C. affords a homogeneous somewhat dough-like solid. If desired, mixing may be carried out under reduced pressure in order to remove any moisture present in the raw materials.

Burning rate test strips of the gas-forming composition are prepared by extruding or molding the homogeneous gas-forming composition at a temperature below about 120° C. under a pressure of about 2000 p.s.i., the test strands being  $\frac{1}{4}$ " to  $\frac{3}{8}$ " in diameter and about 5" long. The strands are coated with lacquer grade cellulose acetate and burned in a Crawford bomb under nitrogen pressure. Four to six strands are burned at varying pressures between 600 and 1800 p.s.i. Plotting burning rate in inches per second against pressure on log-log paper gives a straight line. The slope of this straight line is defined as the exponent of the burning rate as related to pressure in the formula

$$B = \beta \left( \frac{p}{1000} \right)^n$$

where  $B$  is the linear burning rate at pressure  $p$ ,  $\beta$  is the linear burning rate for the composition at 1000 p.s.i.,  $p$  is pressure in p.s.i. in the burning chamber and  $n$  is the pressure exponent showing dependence of the burning rate on pressure. This relationship of burning rate and pressure is discussed by R. N. Wimpress in "Internal Ballistics of Solid Fuel Rockets" (1950).

Gas-producing grains are prepared from the above compositions containing ammonium nitrate, combustion catalyst and binder material by molding under a pressure of about 2000 to 4000 p.s.i. The size and shape of the

grains are dependent upon their intended use. Grains are provided with centrally located holes of different shapes, that is, starform, cruciform or circular. Each grain has the external surface inhibited by a coating of a material such as asphalt to restrict burning to the internal surface. Test grains subjected to tests described hereinbelow and for use in a test motor, which grains were 2.75" in diameter and about 4" in length, were provided with a starform centrally located hole. The test data obtained by burning such grains in the test motor indicate overall performance of the compositions when used in assist take-off operations. For these operations the grains are mounted in a conventional case provided with a suitably placed igniter charge such as cannon powder, which is fired electrically. The igniter flame in turn ignites the propellant grain. The temperature of the gases produced by burning of grains may be of the order of 1500° F. to 3400° F. and the pressure or impulse produced by the hot gases will be dependent upon the grain size, diameter of the nozzle, and other factors. The gas-producing grains may be molded into disc-form, stacks of discs being used as gas-forming propellant material for missile rockets.

As indicated hereinabove, the grains of diameter 2.75" in length are given a thermal shock test which is referred to herein as the cycling test. In this test, grains of a given composition are held in an oven at a temperature of 175° F. for a period of two hours, following which the grains are immediately subjected for a period of two hours to a temperature of -75° F. to complete one cycle. After a second cycle, the grains are permitted to come to room temperature, i.e., about 75° to 80° F. These grains are examined for indications of cracking, crystallinity, and resistance to deformation and shattering when dropped on a concrete surface. Grains are then fired at -75° F., 175° F. and normal ambient temperatures following the cycle treatment. In general, grains made with the plasticized polyvinyl acetate of this invention show no physical defects following the thermal cycling test, and show firing qualities after the cycling test identical with grains which have not been submitted to the high and low temperature cycles.

Another test to which finished grains are subjected is that of hot aging. In this test, grains are stored in an oven at 170° F. in the presence of circulating air. Several grains of a given composition are used in such a test. Grains are withdrawn periodically and tested with respect to firing and burning qualities. The best grains will not be affected after 30 days or more of high temperature storage. A grain which will not tolerate prolonged hot storage malperforms ballistically. It may give an erratic time-pressure curve and may sometimes even burn with explosive violence. In general, the ammonium nitrate grains made up with the plasticized polyvinyl acetate of this invention are superior with respect to burning performance after hot aging.

The "135° C. gas stability test" which is a measure of the chemical stability and gassing properties of the propellant composition is carried out as follows:

Three grams of a finely divided ammonium nitrate gas-forming composition is placed in a vessel. The vessel is connected by tubing to a mercury manometer system which is so arranged that differential readings of the manometer are translatable into volume changes in the system. Since the volume change of the sample itself can be disregarded, the volume change in the system corresponds to the amount of gaseous decomposition products of the sample. The vessel is inserted to an opening in a metal block: this metal block is provided with electrical heating elements and with controls which permit the block to be maintained at a temperature of 135° C. A period of 15 minutes is allowed for the sample to come to the temperature of 135° C. At this time the manometer is zeroed. Readings are taken at 15-minute intervals until the gassing rate is substantially constant. The

manometer readings are converted to cc./g./hr. for each interval. This rate is plotted against the time of heating. In general, it is considered that a composition which has a zero gassing rate during the first hour of heating will be substantially free of gassing tendency in storage at atmospheric temperatures. The compositions of this invention consisting of defined binder, ammonium nitrate, an inorganic catalyst and an alkaline-reacting inhibitor exhibit extremely low gassing rates in this test. Even the presence of finely divided carbon does not render the composition unsatisfactory with respect to storage stability at elevated temperatures.

The following examples are illustrative of propellant compositions which may be used in the propelling of rockets and in assist takeoff operations as described above.

*Example 1*

A binder material for an ammonium nitrate gas-forming composition was prepared by mixing at a temperature of about 120° C., 35 parts by weight of polyvinyl acetate with a molten mixture consisting of 45 parts by weight of 2,4-dinitrodiphenyl ether and 20 parts by weight of 2,4-dinitrotoluene. The mixture was stirred to form a homogeneous plasticized mass. This binder material was tough and rubbery at ambient temperatures. A plasticized ammonium nitrate gas-producing propellant composition consisting on a weight basis of 74% finely ground ammonium nitrate, 23% of the above binder, and 3% insoluble Prussian blue catalyst was formulated by mixing to homogeneity at a temperature of about 100° C. A  $\frac{1}{4}$ " diameter test strand of the finished composition was extruded at a temperature of about 100° C. and a pressure of 2000 p.s.i. This test strip had a burning rate of 0.12 inch per second at 1000 p.s.i. and the pressure exponent was 0.72.

*Example 2*

A thermoplastic binder material consisting of 25% by weight of polyvinyl acetate described in Example 1 and 75% by weight of bis(2,4-dinitrophenyl)-triglycol ether was prepared. This binder was used to formulate a plasticized gas-producing ammonium nitrate composition. The bis(2,4-dinitrodiphenyl)-triglycol ether was prepared by reacting 2,4-dinitrochlorobenzene with triethylene glycol in mol ratio of 2 to 1 using 50% aqueous sodium hydroxide at a temperature of 105-110° C. The binder material was prepared according to the procedure of Example 1. It was rubbery and moderately tough. A gas-forming propellant composition was prepared from the above binder by adding at 95°-105° C. a mixture of finely ground ammonium nitrate, finely divided carbon in the form of Micronex (Standard) beads, and insoluble Prussian blue, and mixing the components to homogeneity. The composition consisted of:

| Component:                              | Percent by weight |
|-----------------------------------------|-------------------|
| Ammonium nitrate                        | 76                |
| Bis(2,4-dinitrodiphenyl)triglycol ether | 15                |
| Polyvinyl acetate                       | 5                 |
| Prussian blue catalyst                  | 3                 |
| Carbon                                  | 1                 |

A screw-extruded strand of this composition showed a burning rate of 0.18" per second at 1000 p.s.i. and a pressure exponent of 0.62.

*Example 3*

A thermoplastic polyvinyl acetate binder was made in a steam-heated mixer according to the method of Example 1 except that triethylene glycol di-2-ethylhexoate, a commercial plasticizer known as Flexol 3GO, was substituted for the dinitrotoluene component. The polyvinyl acetate was Gelva-800. The binder consisted of 40% polyvinyl acetate, 30% 2,4-dinitrodiphenyl ether and 30% Flexol 3GO, and was rubbery and moderately tough. A propellant mixture was made with this binder at about 100° C. Total mixing time was one hour, including 20 minutes of vacuum mixing at 20-25". In preparing the propellant

the binder was first softened in the mixer. Finely ground ammonium nitrate admixed with insoluble Prussian blue, carbon black in the form of Micronex beads (Standard), urea and diphenylamine were added and mixed to homogeneity with the binder at a temperature of 95°-105° C. The composition of this propellant composition was:

| Component:       | Percent of weight |
|------------------|-------------------|
| Binder           | 12.0              |
| Prussian blue    | 3.0               |
| Carbon           | 1.0               |
| Diphenylamine    | 0.8               |
| Urea             | 0.8               |
| Ammonium nitrate | 82.4              |

A part of this propellant composition was molded in the form of 2.75" star grains at 2000 p.s.i. A 4" length star grain was fired successfully after being subjected successively to temperatures of -75° F. and 175° F. in the thermal cycling test described above. Another 4" star grain was "aged" for 70 days at 170° F. during which period it lost about 1% in weight. This aged grain burned smoothly in a rocket motor at a pressure of 1000 p.s.i. using a nozzle of 0.20" diameter.

Another binder consisting of 40% polyvinyl acetate, 25% Flexol 3GO and 20% 2,4-dinitrodiphenyl ether was prepared. A gas-producing propellant composition was formulated according to the procedure outlined in Example 1 by mixing with the binder material finely divided ammonium nitrate containing admixed therewith equal amounts of diphenylamine and urea stabilizer, finely divided carbon in the form of Micronex beads and a small amount of surfactant, that is, 0.1% (based on the weight of the formulation) of the commercial product "Span 85" which is sorbitan trioleate. The gas-forming composition consisted of 79.9% ammonium nitrate, 5.6% polyvinyl acetate<sup>1</sup>, 5.6% Flexol 3GO, 2.8% 2,4-dinitrodiphenyl ether, 1.5% insoluble Prussian blue catalyst, 1.5% ammonium dichromate catalyst, 1% diphenylamine, 1% urea, 1% finely divided carbon and 0.1% sorbitan trioleate. The material was molded to form 2.75" star grains and also to form burning test strips. Grains of 4" length were cycled and these fired successfully following this test. After 36 days of hot storage (170° F.) these grains showed weight loss of less than 0.2%. The burning rate of test strands was 0.11 inches per second at 1000 p.s.i. and the pressure exponent was 0.60.

*Example 4*

A thermoplastic polyvinyl acetate binder was prepared in a steam-heated mixer according to the method of Example 3 from polyvinyl acetate<sup>1</sup> (40%), 2,4-dinitrodiphenyl ether (30%), and Flexol 3GH (30%). The binder was rubbery and tough and was used in formulating the following gas-forming ammonium nitrate compositions according to the method described in Example 3.

| Component:                      | Wt. percent |
|---------------------------------|-------------|
| Polyvinyl acetate               | 4.8         |
| DNDPE <sup>2</sup>              | 3.6         |
| Flexol 3GH                      | 3.6         |
| Prussian blue                   | 3.0         |
| Carbon black <sup>3</sup>       | 1.0         |
| NH <sub>4</sub> NO <sub>3</sub> | 84.0        |

| Component:                      | Wt. percent |
|---------------------------------|-------------|
| Polyvinyl acetate               | 4.8         |
| DNDPE <sup>2</sup>              | 3.6         |
| Flexol 3GH                      | 3.6         |
| Prussian blue                   | 3.0         |
| Carbon black <sup>3</sup>       | 1.0         |
| Magnesium oxide                 | 1.0         |
| NH <sub>4</sub> NO <sub>3</sub> | 83.0        |

<sup>1</sup> Gelva-800.

<sup>2</sup> 2,4-dinitrodiphenyl ether.

<sup>3</sup> Micronex beads (Standard).

9

4c

| Component:                | Wt. percent |
|---------------------------|-------------|
| Polyvinyl acetate         | 4.8         |
| DNDPE <sup>1</sup>        | 3.6         |
| Flexol 3GH                | 3.6         |
| Ammonium dichromate       | 3.0         |
| Carbon black <sup>2</sup> | 1.0         |
| Ammonium nitrate          | 84.0        |

4d

| Component:                | Wt. percent |
|---------------------------|-------------|
| Polyvinyl acetate         | 4.8         |
| DNDPE <sup>1</sup>        | 3.6         |
| Flexol 3GH                | 3.6         |
| Ammonium dichromate       | 3.0         |
| Carbon black <sup>2</sup> | 1.0         |
| Magnesium oxide           | 1.0         |
| Ammonium nitrate          | 83.0        |

4e

| Component:                | Wt. percent |
|---------------------------|-------------|
| Polyvinyl acetate         | 4.8         |
| DNDPE <sup>1</sup>        | 3.6         |
| Flexol 3GH                | 3.6         |
| Ammonium dichromate       | 1.0         |
| Prussian blue             | 2.0         |
| Carbon black <sup>2</sup> | 1.0         |
| Magnesium oxide           | 1.0         |
| Ammonium nitrate          | 83.0        |

<sup>1</sup> 2,4-dinitrodiphenyl ether.<sup>2</sup> Micronex beads (Standard).

Formulation 4a showed excessive gassing after 15 minutes at 135° C. Formulation 4b showed no gassing during 7 hours after which the gassing rate was extremely low.

Test strands of the above compositions were molded at 2000 p.s.i. and burned in the Crawford bomb. The results are tabulated below:

| Formulation | Burning Rate,<br>Inches/Sec. at<br>1,000 p.s.i. | Pressure<br>Exponent |
|-------------|-------------------------------------------------|----------------------|
| 4a          | 0.16                                            | 0.60                 |
| 4b          | 0.15                                            | 0.65                 |
| 4c          | 0.14                                            | 0.49                 |
| 4d          | 0.12                                            | 0.42                 |
| 4e          | 0.16                                            | 0.51                 |

Comparing 4e with a, b, c and d indicates that the use of a catalyst consisting of both Prussian blue and ammonium dichromate, together with magnesium oxide offers advantages with respect to both burning rate and pressure exponent.

#### Example 5

A binder material was prepared according to the procedure described in Example 1 by adding polyvinyl acetate (40%) i.e., Gelva-800, mixture of diethyl phthalate (30%), 2,4-dinitrodiphenyl ether (10%) and bis(2,4-dinitrophenyl) polyglycol 200 ether (20%). The bis(2,4-dinitrophenyl) polyglycol 200 ether was prepared according to the following procedure: A mixture of 1275 grams (6.3 mols) of a commercial grade 2,4-dinitrochlorobenzene and 629 grams (3.1 mols based on a molecular weight of 200) of polyethylene glycol 200 was stirred to obtain an intimate mixture. To this mixture was added dropwise 284 grams of sodium hydroxide dissolved in 300 milliliters of water over a period of 45 minutes. The temperature of the reaction mixture was maintained between 105°-112° C. and was stirred for an additional one and one half hours following which the reaction mixture was added to about 3800 milliliters of water with stirring. The washed oil product was separated from the wash water and the washing procedure was repeated five times, the last wash water being made slightly acid with dilute hydrochloric acid. The product was dissolved in benzene and the residual water was removed by distillation with

10

the benzene in vacuo at 100° C. and 2 mm. pressure. The ash content of the product was 0.12%. The nitrogen content was 10.51%. Calculated nitrogen content was 10.61%.

5 The binder material prepared with the polyvinyl acetate plasticized with diethyl phthalate, 2,4-dinitrodiphenyl ether, and bis(2,4-dinitrophenyl) polyglycol 200 ether was rubbery and moderately tough.

In preparing the ammonium nitrate gas-forming composition, 85.4 parts by weight of finely divided ammonium nitrate was intimately mixed with 1.5 parts by weight of insoluble Prussian blue catalyst, 1.5 parts by weight of ammonium dichromate, 1 part by weight of finely divided carbon in the form of Micronex beads, 0.75 parts by weight of diphenylamine and 0.75 parts by weight of urea. These were also added to the ammonium nitrate 0.1 part by weight of Arlacel C surfactant i.e., sorbitan sesquioleate, and the mixture of ammonium nitrate, binder and other components was stirred to homogeneity at about 100° C.

The composition of the gas-forming ammonium nitrate propellant on a weight basis was: polyvinyl acetate, 3.6%, diethyl phthalate 2.7%, dinitrodiphenyl ether, 0.9%; bis(2,4-dinitrophenyl) polyglycol 200 ether 1.8%, Prussian blue 1.5%, ammonium dichromate 1.5%, carbon 1%, diphenylamine 0.75%, urea 0.75%, surfactant 0.1%, and ammonium nitrate 85.4%. A part of this composition was molded into burning strands. Cylindrical propellant grains having a diameter of 2.75" and provided with a star-shaped internal aperture, were molded, at about 2000 pounds per square inch pressure. Some of these grains were cycled in the thermal cycling test and were fired successfully in the test motor following the cycling test. Another of these grains was fired successfully after being subjected to a storage temperature of 170° F. for a period of 13 days. The motor burning rate was about 0.18 inch per second at 1000 p.s.i.

#### Example 6

40 A binder material consisting of polyvinyl acetate (40%), 2,4-dinitrodiphenyl ether (10%), triethylene glycol di-2-ethylbutyrate (20%), (Flexol 3GH) and 2,4-dinitrophenyl propyl ether (30%) was prepared according to the method described in Example 1. The binder was moderately tough and rubbery. The 2,4-dinitrodiphenyl ether and the 2,4-dinitrophenyl propyl ether were prepared according to the method described in the above application S.N. 465,132, normal propyl alcohol being substituted for the phenol in the preparation of the 2,4-dinitrophenyl propyl ether. This binder was used in preparing a solid propellant mixture in the manner described in Example 5.

The finished composition contained on a weight basis, the following:

| Component:                | Wt. percent |
|---------------------------|-------------|
| Ammonium nitrate          | 81.0        |
| Binder                    | 14.0        |
| Ammonium dichromate       | 2.0         |
| Prussian blue             | 1.0         |
| Micronex beads (Standard) | 1.25        |
| Magnesium oxide           | 0.75        |

The finished composition was molded into cylindrical grains having a diameter of 2.75". Nine motor firings were made on cycled grains. Three at -75° F., three at ambient temperatures and three at 175° F. The grains showed uniformly satisfactory firing behavior in the test motor using a 0.222"-30° nozzle. The grains were particularly resistant to physical shock. One of the cycled grains was dropped from a height of eight feet onto concrete and then was fired successfully in the test motor. The grains were also subjected to hot storage at 170° F. and fired satisfactorily following 30 days storage at this temperature. Burning tests made with molded

strands indicated a burning rate of 0.15" per second at 1000 p.s.i. and a pressure exponent of 0.47.

Percentage compositions in this specification and claims based thereon are percentages by weight unless indicated otherwise.

Having thus described my invention, I claim:

1. A gas-forming composition consisting essentially of (a) between about 70 and about 90 weight percent of ammonium nitrate, (b) between about 1 and 5 weight percent of an inorganic combustion catalyst selected from the class consisting of ammonium dichromate and Prussian blue, (c) between about 5 and 25 weight percent of plastic binder material, said material consisting of (i) between about 20 and 60 weight percent of polyvinyl acetate and (ii) a plasticizer selected from the class consisting of (I) nitro-substituted aromatic compounds corresponding to the formula



where R is selected from the class consisting of nitrophenyl, phenoxy, mononitrophenoxy and alkoxy containing from 1 to 4 carbon atoms, (II) nitrophenyl glycol ether wherein said glycol-portion affording compound has a molecular weight of not more than about 200 and (III) mixtures of said nitro-substituted aromatic compounds selected from I and II with a member selected from the class consisting of dialkyl phthalates, triethyl citrate, tributyl citrate, diethyl tartrate, dibutyl tartrate, triglycol dialkanoates, polyglycol dioctanoate, dialkyl diglycolates, dinitrobenzene and dinitrotoluene, said mixture containing at least about 30 weight percent of said nitro-substituted aromatic compounds and (d) between

about 0.2 and 3 weight percent of an alkaline gassing inhibitor from the class consisting of diaminobenzene, diphenylamine, urea and magnesium oxide.

2. The composition as described in claim 1 wherein 5 the inorganic catalyst consists of a mixture of insoluble Prussian blue and ammonium dichromate.

3. The composition as described in claim 1 wherein the inorganic catalyst consists essentially of insoluble Prussian blue.

10 4. The composition of claim 1 to which is added from about .5 to about 2% of finely divided carbon.

5. The composition as described in claim 1 to which is added from about 0.2 to about 3% by weight of magnesium oxide.

15 6. A shaped gas-forming grain consisting essentially on a weight basis, of ammonium nitrate, about 81%, insoluble Prussian blue about 1%, about 2% of ammonium dichromate, about 5.6% polyvinyl acetate of viscosity of 700 to 900 centipoises at 20° C., 2,4-dinitrodi- 20 phenyl ether about 1.4%, 2,4-dinitrophenyl propyl ether about 4.2% and triethylene glycol di-2-ethylbutyrate about 2.8%, about 1.25% of carbon black and about 0.75% of magnesium oxide.

25 **References Cited in the file of this patent**

**UNITED STATES PATENTS**

2,159,234 Taylor ----- May 23, 1939

**FOREIGN PATENTS**

30 655,585 Great Britain ----- July 25, 1951

**OTHER REFERENCES**

35 Bebie: "Manual of Explosives, Military Pyrotechnics and Chemical Warfare Agents," The MacMillan Co., New York (1943), pages 57, 58, 60, 61, 62.